

## UNITED STATES PATENT OFFICE

2,440,526

## FIBROUS SHEET MATERIAL FOR THE ELECTROLYTIC FORMATION OF AN AZO DYE-STUFF THEREON

Myer Solomon, deceased, late of Westmont, N. J.,  
by Nellie W. Solomon, administratrix, Princeton,  
N. J., assignor to Radio Corporation of America, a corporation of Delaware

No Drawing. Application December 23, 1942,  
Serial No. 469,958

8 Claims. (Cl. 204—2)

1

This invention relates to the art of electrolytic dye production and more particularly, to an article of manufacture involving a fibrous sheet material for the electrolytic formation of azo dyestuffs thereon. In a preferred adaptation, it includes the production of dyes of the aforementioned type in connection with the art of facsimile recording. The fundamentals of the present disclosure are set forth in the copending application Serial No. 178,743, now U. S. P. 2,306,471, of which earlier application the present application is a continuation-in-part.

Various types of facsimile receivers are used at the present time, and in substantially all of them pictures, printed matter, or other characters are produced on a recording sheet of paper in response to variations in electrical current which are received from the transmitter station. In one type the reproduction of the character or indicia is through the use of carbon paper and the transfer of the carbon to the record paper is accomplished by means of an electromagnetically controlled printer bar. In such a device the recording paper and carbon paper are placed in the facsimile receiver and are moved forward at rates which are necessarily slow because of mechanical inertia limitations, while line increments of the material being received are reproduced through the application of varying degrees of pressure to the printer bar, in order that varying amounts of the carbon will be transferred from the carbon paper to the recording paper. Such a device for facsimile recording is shown in the patent to Charles J. Young, Reissue #20,152, October 27, 1936.

In another type, a light sensitive recording paper is used and the amount of light permitted to strike the paper is controlled in accordance with the electrical variations transmitted by the facsimile transmitting device. In this type some developing or fixing process generally follows.

In still another type a stream of hot air is directed against a heat responsive recording paper, the intensity of the heat or the amount of hot air being controlled in response to the energy transmitted by the facsimile transmitting device. Another type uses a jet of ink or some colored

2

fluid, the jet being permitted to strike, or being prevented from striking, the recording paper according to the series of signals received from the transmitting device. The patent to Richard H. Ranger, #1,770,493, of July 15, 1930, shows, for example, devices wherein jets of hot air or ink are used for facsimile recording.

In the facsimile receiving or recording systems referred to above, the production of half tones and shades such as occur in the reproduction of pictures, is somewhat difficult, since, for instance, in the carbon paper method, the transfer of the carbon to the recording paper is somewhat critical in response to the pressure applied to the printer bar. Furthermore, the use of hot air or ink jets is not entirely satisfactory since such systems are difficult to control and to maintain in proper operation.

The present invention may be generally characterized as directed to dye formation, in which electrolytic action plays an essential part, and is particularly applicable to electrolytic diazotization and coupling.

It is an object of the invention to overcome the difficulties and limitations of the prior art procedures noted hereinabove.

It is an additional object of the invention to electrolytically produce azo dyes, involving elements of novelty as to composition of matter, article of manufacture, and details of procedure.

It is another object of the present invention to obtain diazonium compounds by the action of an electric current on mixtures or solutions containing diazotizable amines and nitrites.

It is a further object to provide mixtures or solutions containing diazotizable amines and nitrites which are adapted to electrolytically react for the purpose of producing diazonium compounds.

Another object of the invention is to provide solutions or, where feasible, mixtures, of appropriate reagents comprising a diazotizable amine and an ionizable nitrite which are adapted for electrolytic reaction to produce a diazonium compound, and to form azo dyes from such diazonium compound by reaction with a coupling reagent present in said mixture or solution.

Another object of the invention is a novel supporting material or carrier containing dye forming chemical reagents which will react suitably when subjected to electrolytic treatment.

An added object of the invention is a supporting material or carrier treated with azo dye forming chemical reagents which will react suitably when subjected to electrolytic treatment, said carrier as a result of its chemical treatment being electrolytically conductive.

A further object is a supporting material or carrier impregnated with reagents adapted for azo dye formation when subjected to an electric current, and substantially inert to dye formation in the absence of the effect engendered by the electrolytic action.

A still further object of the invention is to provide a supporting surface or carrier which is saturated or impregnated with a diazotizable amine and an ionizable nitrite, which is advantageously adapted for production in situ of a diazonium compound when subjected to an electric current.

An important object of the invention is to provide articles of manufacture adapted for facsimile recording in the form of a carrier or supporting material treated with appropriate chemical reagents for forming a dye electrolytically when subjected to an electric current, said dye formation corresponding with electric impulses emanating from a transmitting source, for example, from a scanning station.

An additional object of the invention is to provide a supporting surface saturated or impregnated with a diazotizable amine, an ionizable nitrite, a coupling reagent, an electrolyte, and other predetermined perfecting ingredients, said supporting surface being thereby adapted for electrolytic facsimile recording through azo dye formation.

Other objects, features and advantages of the invention will be apparent from the following detailed description.

In the present invention, it is proposed to produce the picture of printed matter on the recording paper in the form of an azo dye, the amount of such dye deposited being a function of the amount of current caused to flow through the recording paper. When the image is thus formed, for example, by applicant's electrolytic azo dye formation, the pressure of the printer bar can be maintained constant and the amount of current which is passed through increments of the paper simply varied in accordance with the light and dark portions present on the picture or printed matter being scanned at the facsimile transmitter. When dyes are so formed by electrolytic action, the varying half tone shades may be produced by merely regulating the amount of the current which is caused to flow through the recording paper.

The electrolytic diazotization method contemplated herein can be viewed as deriving from a general concept that mixtures of a diazotizable amine, for example, a suitable primary aromatic amine, and an ionizable nitrite, such as a metal nitrite or the like, are stable in mild alkaline solution, the amino group being un-ionized and the nitrite ion having a negative electric charge, whereby diazotization is substantially precluded and no formation of diazonium salt takes place. Diazotization of these compounds may be effected in the presence of a suitable concentration of hydrogen ions, usually accomplished by supplying an appropriate quantity of acid. In the present invention, the provision of a suitable hydro-

gen ion concentration is brought about by the action of the electric current at the anode in an electrolytic cell, thus causing practically immediate diazotization or diazonium-ion formation in the region of the anode, but not before the reagents are subjected to the electrolytic action in the effective zone of the anode. Stated in another fashion, any premature electrolytic diazotization to produce diazonium compounds in accordance with the present invention, is precluded by maintaining such conditions in the solutions of the amino compound and nitrite reagent that there is no material interreaction until such time as the current is passed through it; as above indicated, this control depends upon the fact that the diazotization reaction will only take place in an acid medium, and this acid medium is made available only in proximity to the anode. The main body of the solution remains fundamentally alkaline or non-acid in character.

Where coupling compounds are present in the reacting mixture, or are added after diazotization occurs, azo dyes are formed under conditions appropriate to the reaction of the coupling reagent with the diazonium compound. Thus, where mixtures containing amines, nitrites, and coupling compounds are subjected to electrolytic diazotization, and the coupling compound is of the acid reacting type, coupling will occur substantially spontaneously within an extremely brief interval after passage of the current which results in the provision of an acid zone adjacent the anode.

While an acid zone is created and prevails adjacent the anode, the zone adjacent the cathode tends to increase in alkalinity as a result of the current passing through the cell existing between the electrodes. The solution as a whole is therefore preponderantly alkaline, despite the presence of hydrogen ions produced in the anode zone and subsequent ionic migration tends to re-establish the original conditions after the electrolysis. Accordingly, where the coupling reagent is of the type which reacts in an alkaline medium, the general alkalinity of the solution will cause the diazonium salt produced adjacent to the anode to couple with the alkaline coupling reagent at any point removed from the anode to form the predetermined dye product. Coupling compounds that react in alkaline solution frequently yield better results, where acid coupling compounds are not sufficiently reactive for the coupling to be completed before the original alkalinity is restored.

Where the compound is of the type which will couple in an alkaline medium, there may of course be a slightly longer time element involved to attain the azo dye formation. This time interval is usually of the order of less than a minute after the passage of the current which causes diazotization. Therefore, while alkaline coupling may require a somewhat longer time interval than that necessitated by reagents which couple in an acid medium, alkaline coupling may, nevertheless, be appropriately classified as spontaneous, similarly to the case of the coupling in an acid medium.

Various regulations of the procedure obviously may be resorted to so that both acid coupling and alkaline coupling may occur during the course of formation of a given azo dye. In general, the appropriate selection can be more or less guided, without limitation thereto, by considering acid coupling as the reaction where a diazonium compound attaches itself to the ring of the coupling compound, replacing the active hydrogen which

becomes a hydrogen ion and alkaline coupling as the reaction where the diazonium compound attaches to the ring of the coupling compound with the displacement of hydrogen and the hydrogen unites with hydroxyl to form water.

Considering the process as applied to a paper recording sheet in facsimile recording, as will be further considered hereinbelow, when a point on the paper is between the electrodes, positive electric current causes acidification and diazonium ion formation. Acid coupling immediately starts. When said point on the paper moves away from the point of contact with the electrodes, the current ceases and the excess acid on the + side begins to be neutralized by the excess alkali on the - side so that the rate of acid coupling diminishes and alkaline coupling starts. During the time that both sides of the paper are regaining their original alkalinity, the acid coupling rate becomes very slow and alkaline coupling accelerates, and usually all of the diazonium compound in the recorded area couples before the paper dries. In general, amino and hydroxy groups direct coupling under acid and alkaline conditions, respectively. Thus, it is possible for both acid and alkaline coupling to be manifested in a given reaction leading to azo dye formation.

Without intending to be restricted to any of the theoretical explanations provided hereinabove or to any suggestions as to the character of the reactions involved therein, or in the azo dye formation generally, it will be noted that an explanation in the form of equations involving the production of diazonium salt electrolytically, and the coupling of this salt, in accordance with the preferred invention embodiments, is presented in U. S. Patent 2,306,471, referred to above.

As previously stated, the preferred procedure in accordance with the present invention comprises adapting the solution for facsimile recording by electrolytically diazotizing an amine, in an alkaline solution which contains an alkaline acting coupling reagent.

The ingredients utilized in accordance with the invention, and especially in its adaptation to facsimile recording, comprise the following:

- (a) An aromatic amine, desirably a primary amine.
- (b) A nitrite.
- (c) An alkali.
- (d) A coupling compound.
- (e) An electrolyte.
- (f) Water or other solvent in which electrolytes ionize.

Concerning the amines required for producing the diazonium compound, substantially any diazotizable amino compound will suffice. Mainly within the purview of such class of compounds are the primary aromatic amines, and especially where the latter are soluble in mildly alkaline salt solution, and are not too readily oxidized electrolytically or by air oxidation.

Among the amines which may be utilized are monoamino benzene compounds, polyamino benzene compounds, amino-naphthalene compounds, amino polyphenyl compounds, heterocyclic amines with a nuclear attached primary amino group such as the amino quinolines, amino pyridines and amino pyrimidines. The presence of a sulphonate group in such amines tends to enhance the stability of the background of the carrier towards light although the dye may, in some cases, manifest somewhat less fastness to washing. Typical illustrative sulphonates are the sulphonic acids of amino-benzene, -naphtha-

lene, or -diphenyl compounds and various amino naphthol sulphonic acids.

The following are illustrative lists of amines and coupling compounds which may be utilized:

#### AMINES

##### *Monoamino benzene compounds*

- 10 1. Sodium formanilide
- 2. Aniline omega-sulphonic acid
- 3. 4-aminoacetophenone
- 4. 4-aminoacetophenoneoxime
- 5. Anthranilic acid
- 6. 4-aminobenzoic acid
- 7. 3-aminobenzoic acid
- 8. Metanilic acid
- 9. Sulphanilic acid
- 10. 2,5-dichlorosulphanilic acid
- 11. 2-aminotoluene-5-sodium sulphonate
- 20 12. 4-aminotoluene-2-sulphonic acid
- 13. Orthonitroanilineparasulphonic acid
- 14. Paronitroanilineorthosulphonic acid
- 15. Paraaminobenzophenone
- 16. Paraaminobenzophenoneoxime
- 17. Metaaminophenol<sup>1</sup>
- 18. 5-aminosalicylic acid hydrochloride
- 19. Orthoaminophenolparasulphonic acid
- 20. 2-amino-4-chlorophenol-6-sulphonic acid
- 21. Orthoaminodiphenylparasulphonic acid
- 30 22. Acetoacetanilide oxime parasulphonic acid<sup>2</sup>
- 23. 1-methaaminophenyl-3-carboxy-5-pyrazolone<sup>1</sup>
- 24. Hydroxylamine with No. 23<sup>1</sup>
- 35 25. Acetoacetanilide hydrazone parasulphonic acid

##### *Polyamino benzene compounds*

- 40 (1) All amino groups on the same benzene ring.
- 26. Orthophenylenediamine<sup>1</sup>
- 27. Metaphenylenediamine<sup>1</sup>
- 28. Paraphenylenediamine<sup>1</sup>
- 29. Chloroparaphenylenediaminedihydrochloride<sup>1</sup>
- 30. 2,5-diaminobenzenesulphonic acid dihydrochloride<sup>1</sup>
- 31. 2,4-diaminotoluene<sup>1</sup>
- 50 32. 2,5-diaminotoluenedihydrochloride<sup>1</sup>
- 33. 2,4-diaminoanisole dihydrochloride<sup>1</sup>
- 34. 2,5-diaminoanisole dihydrochloride<sup>1</sup>
- 35. Triaminotoluene trihydrochloride<sup>1</sup>
- 36. Metaaminoacetanilide dihydrochloride
- 37. Paraaminoacetanilide
- 55 38. Paraaminomethylacetanilide
- 39. Oxalylparaphenylenediamine
- 40. Paraaminodiphenylaminosulphonic acid
- 41. Paraaminophenylparatolylaminosulphonic acid

- 60 (2) At least two amino groups on different benzene rings.

- 65 42. Benzidine
- 43. Dianisidine
- 44. "Solvabilized" dianisidine
- 45. Benzidinemonsulphonic acid
- 46. Benzidine-2,2'-disulphonic acid
- 47. Benzidine-3,3'-disulphonic acid
- 70 48. Orthotolidine-2,2' or -6,6'-disulphonic acid
- 49. 4,4'-diaminobenzophenone
- 50. 4,4'-diaminobenzophenoneoxime
- 51. 4,4'-diaminostilbene-2,2'-disulphonic acid
- 52. 4,4'-diaminodiphenylaminosulphonic acid

*Naphthalene compounds*

53. Orthonaphthionic acid  
 54. Sodium naphthionate  
 55. Laurent's acid  
 56. Cleve's 1.6 and 1.7 acids  
 57. Cleve's 1.6 sulphonic acid  
 58. Peri acid  
 59. Disulpho S salt  
 60. Koch's acid  
 61. 4-acetylaminio-1,7-Cleve's acid  
 62. Tobias acid  
 63. Dahl's acid  
 64. Broenner's acid  
 65. Amino F acid  
 66. Badische acid  
 67. Amino R acid  
 68. Acid IV or C acid  
 69. 2-naphthylamine-5,7-disulphonic acid  
 70. Amino G acid  
 71. Naphthalin Red  
 72. 1-2-4 acid  
 73. J acid<sup>1</sup>  
 74. M acid<sup>1</sup>  
 75. Gamma acid<sup>1</sup>  
 76. S acid<sup>1</sup>  
 77. Chicago or 2S acid<sup>1</sup>  
 78. Monosodium H salt<sup>1</sup>  
 79. K acid<sup>1</sup>  
 80. 2R acid (oxyamino)<sup>1</sup>  
 81. R acid (oxyamino)<sup>1</sup>

*Heterocyclic compounds*

82. 2,6-diaminopyridine
- <sup>1</sup>

*COUPLING COMPOUNDS**Benzene compounds*

83. Resorcinol  
 84. 4-chlororesorcinol  
 85. 2-nitroresorcinol  
 86. Salicylaldehyde  
 87. Salicyaldoxime  
 88. 5-chlorosalicylaldehyde  
 89. 5-chlorosalicyaldoxime  
 90. Orthohydroxybenzalacetophenone  
 91. Orothhydroxybenzalacetophenoneoxime  
 92. Resorcytaldehyde  
 93. Resorcyaldoxime  
 94. Resorcylic acid  
 95. Parahydroxyacetophenone  
 96. Parahydroxypropiophenone  
 97. Resacetophenone  
 98. Resacetophenoneoxime  
 99. Phloroglucinol  
 100. Metaaminophenol  
 101. Acetoacetanilide  
 102. Isonitroscacetacetanilide  
 103. Isonitrosoacetacetanilideoxime  
 104. Acetoacetanilideoxime  
 105. Acetoacetanilide hydrazone  
 106. 2-chloroacetacetanilide  
 107. 2-chloro-isonitrosoacetacetanilide  
 108. 2,5-dichloroacetacetanilide  
 109. 2,5-dichloro-isonitrosoacetacetanilide  
 110. Acetoacetanilide-parasulphonic acid

<sup>1</sup> These chemicals may act both as amines and as coupling compounds. Usually, when involved in diazotization and coupling reactions, some molecules of these compounds act as amines, others as coupling compounds, and the remainder in both capacities, forming mixtures of azo dyes. Many of the other amines, particularly in the naphthalene series, will act also as coupling compounds if no hydroxy coupling compounds are present.

<sup>2</sup> This acts as an amine, although it does not contain an amino group.

111. Acetoacetanilide oxime parasulphonic acid  
 112. 1-metaminophenyl - 3 - carboxy-5-pyrazolone  
 113. Hydroxylamine with No. 112  
 5 114. Acetoacetanilide hydrazone parasulphonic acid  
 115. Orthophenylenediamine  
 116. Metaphenylenediamine  
 117. Paraphenylenediamine  
 10 118. Chloroparaphenylenediaminedihydrochloride  
 119. 2,5-diaminobenzenesulphonic acid dihydrochloride  
 120. Diacetoacetyl-paraphenylenediamine  
 15 121. Diisonitrosodiacetacetyl - paraphenylenediamine  
 122. Diacetoacetyl - paraphenylenediaminedioxime  
 123. 2,4-diaminotoluene  
 20 124. 2,5-diaminotoluenedihydrochloride  
 125. 2,4-diaminoanisole dihydrochloride  
 126. 2,5-diaminoanisole dihydrochloride  
 127. Triaminotoluenetrihydrochloride  
 128. 4,4'-dihydroxybenzophenone  
 25 129. 4,4'-dihydroxybenzophenoneoxime  
 130. Metadiethylaminophenol  
 131. Metadigallic acid (tannic acid)

*Naphthalene compounds*

- 30 132. Alpha naphthol  
 133. Alpha hydroxynaphthoic acid  
 134. Schaeffer's alphanaphtholsulphonic salt  
 135. Neville and Winther's acid  
 136. L acid  
 35 137. N-phenyl Peri acid  
 138. RG acid  
 139. Andresen's acid  
 140. Schoellkopf's acid  
 141. Oxy Koch acid  
 40 142. Beta naphthol  
 143. Beta hydroxynaphthoic acid  
 144. Naphthalin OA  
 145. Schaeffer's acid  
 45 146. F salt  
 147. Bayer's or Crocein salt  
 148. Disodium R salt  
 149. Disodium G salt  
 150. Naphthoresorcinol  
 50 151. 1,5-dihydroxynaphthalene  
 152. 1,7-dihydroxynaphthalene-4-sulphonic acid  
 153. Dioxy S acid  
 154. Nigrotic acid  
 155. Yellow acid  
 55 156. Red acid  
 157. A acid  
 158. Chromotropic salt or acid  
 159. 2,7-dihydroxynaphthalene  
 160. Phenyl J acid  
 60 161. Benzoyl J acid  
 162. Di J acid urea  
 163. J acid imide  
 164. J acid  
 165. M acid  
 65 166. Gamma acid  
 167. Phenyl gamma acid  
 168. S acid  
 169. Chicago or 2S acid  
 170. Monosodium H salt  
 70 171. Chloro H acid  
 172. Phenyl H acid  
 173. Acetyl H acid  
 174. K acid  
 175. 2R acid (oxyamino)  
 75 176. R acid (oxyamino)

*Miscellaneous compounds*

177. 8-hydroxyquinoline  
 178. 8-hydroxyquinoline-5-sulphonic acid  
 179. Barbituric acid  
 180. Violuric acid  
 181. Hydroxylamine with 179  
 182. Thiobarbituric acid  
 183. Thiovioluric acid  
 184. 1-phenyl-3-methyl-5-pyrazolone  
 185. 1-parasulphophenyl-3-methyl-5-pyrazolone  
 186. Hydroxylamine with 185  
 187. 1-parasulphophenyl - 3 - carboxy-5-pyrazolone  
 188. 2,6-diaminopyridine  
 189. Diacetoacetyl ethylenediamine  
 190. Monoisonitrosodiacetylethylenediamine  
 191. Diisonitrosodiacetylethylenediamine  
 192. Monoisonitrosodiacetylethylene diamine oxime  
 193. Monoisonitrosodiacetylethylenediamine oxime  
 194. Diisonitrosodiacetylethylenediamine oxime  
 195. Diisonitrosodiacetylethylenediamine dioxime

Relative to the proportioning of the ingredients, as a general rule by way of estimate and not restriction, approximately 0.03 gram molecular weights (0.015 for diamines) of amine and of a mono-valent nitrite per liter of solution produce quite satisfactory results. Usually 0.025 gram molecular weights or mols of amine are used per liter of solution for paper that is treated at the recorder, that is, for paper which is subjected to the diazotizable solution substantially at the time that the recording is made.

A comparatively wide range of nitrites are available, the requisite being an ionizable compound, desirably a metallic nitrite. Whereas the examples herein involve the use of sodium nitrite, it should be clear that this compound is referred to merely as illustrative of a convenient material which may be utilized in the diazotization procedure. While nitrite sodium provides entirely satisfactory results, the same may be said of potassium nitrite as well as of many other metallic nitrites. In view of the fact that neutral or alkaline solutions of sodium nitrite are comparatively stable, this reagent is particularly desirable in recording solutions prepared for storage over a substantial period prior to usage.

It has been found that excess nitrite does not impair the background permanence of electrolytic diazotization recordings and is in fact beneficial because it causes a greater percentage of the amine to be diazotized, and consequently permits a decrease in the concentration of amine with no loss in color intensity. Concentrations of 0.025 and 0.05 gram molecular weights of amine and of nitrite, respectively, per 1000 cc. of solution, usually give excellent results.

Similarly, a substantial latitude in choice of alkaline reagent is available, but for purposes of illustration herein, recourse is had to sodium hydroxide. The usual content of sodium hydroxide may be characterized as that required to neutralize all strongly acid groups in the amines and coupling compounds, and to provide a slight excess (usually 20 cc. of normal NaOH per liter or recording solution).

Where the alkalinity pertains to the recording solution and is not particularly critical, simple expedients for its approximate evaluation are available in the form of the so-called Beckman

instrument or other commercial devices. Similarly, a small piece of LaMotte "Oleo Red B" pH test paper may be immersed in the facsimile recording solution for a few seconds. The alkalinity is satisfactory if the paper turns orange-brown, insufficient if yellow or orange-yellow, and excessive if red. It should be noted that insufficient alkalinity is more harmful than excessive, since it impairs the background permanence; on the other hand, a stronger signal in the form of electrical impulse is required from the amplifier, and half tones are impaired, when the solution is excessively alkaline.

As a general matter, the color intensity at full electric current depends on the alkalinity and the amount of diazonium compound formed. The deepest color is usually formed at a pH of 7.5 to 9 which is not alkaline enough for good background permanence. At a pH of 6 to 7.5, hydroxy coupling is too slow in some cases, and premature non-electrolytic diazotization discolors the paper in others. At the compromise pH range of 9 to 11.5, the color intensity is not sacrificed unduly in order to gain in background permanence.

The diazotizable composition and the treated carrier, such as paper, may be stored a considerable period of time if the solution is moderately strongly alkaline. A pH range of 7.5 to 12.5 is applicable, although best results are obtained within the range of 10.0 and 11.5. As the pH drops, the stability decreases, the tendency of the background to darken on standing increases, and the sensitivity of the reaction increases.

In lieu of sodium hydroxide, other strong bases may be used, such as potassium hydroxide, barium hydroxide, or a quaternary ammonium hydroxide. On a weight basis, the amount of alkali used may vary from 0.01 to 0.12 gram molecular weights per liter of solution, depending upon the original acidity or alkalinity of the other ingredients, and is adjusted to the predetermined pH of the finished solution, which, as above suggested, may desirably be within the range of 10.0 to 11.5.

The coupling compounds are desirably soluble in a mildly alkaline salt solution and preferably subject to the same oxidation limitations as discussed above in connection with the amines. Aromatic compounds with hydroxy, amino or active methylene groups, ortho or para, to unsubstituted positions in the ring will usually couple. Sulphonic groups have the same effect as in amines. Resorcinol, phloroglucinol, the naphthols and their sulphonic acids, 8-hydroxy quinoline, and some amino naphthol sulphonic acids have given good results. Some amino naphthol sulphonic acids (for example, gamma, H, J, S and 2S acids) may either diazotize or couple. Good recordings may thus be obtained, using the same chemical for both diazotization and coupling. However, most amino naphthol sulphonic acids give recordings that require washing in order to prevent the backgrounds from darkening during storage.

Chromotropic salt is considered the best all-round coupling compound, giving darker colors than any of the others having reasonably permanent white backgrounds. The aceto-acetyl-amino compounds, their oximes and hydrazones, and the isoxazolones and pyrazolones derived from them, give yellow or orange colors, the oximes and hydrazones being most effective.

When added to facsimile recording solutions con-

## 11

taining chromotropic salt, these yellow or orange couplers improve the color, giving brownish-purple shades that are more pleasing in appearance than the purple obtained with chromotropic salt alone. The ratio of chromotropic salt to oxime or hydrazone is usually three gram-molecules to one.

The coupling compounds may be utilized individually or in admixture, particularly desirable results being obtainable from the use of a plurality of coupling compounds, as indicated in an example hereinbelow.

The amount of coupling compound utilized may vary between 0.01 to 0.02 gram molecular weights, although more may be utilized without harm. Usually approximately 0.015 gram molecular weights of coupling compound per liter of solution provides excellent results, and a greater amount rarely shows any improvement in recorded color intensity.

As above indicated, the coupling compound may be of the type which reacts in alkaline medium or in acid medium, although the former is preferable. It is interesting to note that some amino compounds may function as coupling agents regardless of the pH, and many diazotizable primary amines serve in the dual function of amine and coupling compound. Under alkaline conditions, the hydroxy-coupling rate of reaction is generally so much greater than the amino coupling rate that substantially little or no amino coupling takes place in alkaline solution when both amino and hydroxy groups are present.

As for the electrolyte, NaCl is quite satisfactory, but there is no intent to be limited to the use of this salt. Other strong neutral electrolytes such as NaBr, KBr, KCl, LiCl, BaCl<sub>2</sub>, CaCl<sub>2</sub>, MgCl<sub>2</sub>, K<sub>2</sub>SO<sub>4</sub>, Na<sub>2</sub>SO<sub>4</sub>, MgSO<sub>4</sub>, etc., may be substituted for sodium chloride. Some dye intermediates are more soluble in potassium chloride solutions, in which cases the substitution is made. Lithium chloride has been found to retard the time of paper drying, but the same result is cheaper and more effectively obtained by the use of wetting agents. An additional electrolyte which has provided excellent recordings, while at the same time obviating the corrosive effect of nascent chlorine, is sodium sulphamate,



The amount of electrolyte required is not critical. Low concentrations require more electric current, while excessively high concentrations may cause partial precipitation of the dye intermediates. About two-thirds of a mol (a mol equals one gram molecular weight) of total electrolyte per liter of solution is fully adequate. For convenience in making the sodium ion correction to the Beckman pH meter readings, a total sodium ion concentration of 0.64 mol is used. The total sodium present in all the other ingredients is subtracted from 0.64, the remainder representing the amount of sodium chloride to be added.

Where NaCl is utilized, it has been found that the total concentration of sodium ions equal to 1.0 gram molecular weight per liter is quite effective, although good recordings have been obtained in some cases with as low as 0.1 and as high as 3.0 gram molecular weights of sodium per liter.

Substitution of sodium oxalate for part of the sodium chloride retards the background darkening of damp pretreated paper, although the elec-

## 12

tric current requirements are increased, and the halftone response is somewhat impaired. Oxalates have little effect on the background permanence of recordings exposed to light after drying, and their use is advisable primarily with damp treated paper.

It is, of course, apparent that water functions as a very desirable and effective solvent within which the diazotization and azo dye formation are carried out. However, various non-aqueous neutral solvents that permit electrolytes to ionize may be substituted for all or a part of the water. If approximately half the water is replaced by alcohols or glycols, the freezing point of the solution is lowered to such an extent that recorders may be operated outdoors in winter.

Ethyl, methyl and isopropyl alcohols evaporate more rapidly than water, so that the paper dries too quickly in summer but in winter the added speed is desirable. Normal propyl alcohol dries at approximately the same rate as water, and may be used both summer and winter. The tendency of the propanol-water-salt mixture to separate into two liquid phases is eliminated by replacing ten per cent of the propanol with ethylene glycol. Larger amounts of the glycols are unsatisfactory, as their low volatility causes the recordings to be permanently limp and moist.

Some solvents, notably Cellosolve, methyl Cellosolve, and most denatured ethyl alcohols, gradually react with the alkali in the recording solution, which eventually becomes acid (unless more alkali is occasionally added), whereupon diazotization and coupling begin, causing paper treated with the solution to become discolored. Normal propyl alcohol and ethylene glycol do not reduce the alkalinity.

It will be noted that auxiliary chemicals are of substantial usage, and contribute materially to the control of the diazotization, dye formation, and recording generally. Such substances as oxalates, antifreeze solvents, hydroxylamine and hydrazine may be considered either as auxiliary chemicals or as replacements for part of the essential chemicals.

An important role may be attached to the use of auxiliary chemicals in connection with the dye formation, and particularly where facsimile recording is concerned. These substances contribute materially to the control of the diazotization, dye formation, and recording generally.

Urea, thiourea, and, to a still greater extent, dicyandiamidine have been found to improve the color intensity. About 1 to 2 mols of either of these compounds per mol of amine are used. This effect is more apparent when combined with that due to excess nitrite. If a sulphate or hydrochloride of these bases is used, sufficient caustic soda or other alkali must be added to liberate the free base, in order to maintain the proper pH range.

Wetting agents may be utilized in the treatment of the carrier, such as paper. Many of such wetting agents and their general field of usage as well as chemical characteristics are set forth in the Journal of Industrial and Engineering Chemistry, volume 31, June 1939, pages 66-69. Wetting agents which have been found quite effective are sulfonated ether (see page 69, volume 31 of Journal of Industrial and Engineering Chemistry, January, 1939) as well as the sodium salts of aryl alkyl poly ether sulfonate (p. 130, volume 35, Journal of Industrial and Engineering Chemistry) and dioctyl ester sodium sulfosuc-

cinic acid (page 126, volume 35, Journal of Industrial and Engineering Chemistry).

The rate of penetration of the dye forming solution into the carrier or supporting material, such as paper, is most rapid at high alkalinity and low surface tension of the solution, as well as at high atmospheric humidity. It is in this connection that wetting agents have been found highly effective in reducing the surface tension sufficiently for adequate wetting to occur in a brief interval of paper submersion time, desirably approximately six seconds, regardless of the humidity and alkalinity prevailing. As an example of the quantity of wetting agent, 0.8 of wetting agent solids per liter of solution has been found to afford adequate wetting when the paper is immersed. Where the paper is supplied with the dye forming solution by contacting only one side of the paper with a wet roller approximately 1.5 grams of wetting agent per liter of solution may be essential.

The desirability of resorting to wetting agents in the recording solutions is emphasized by the fact that without the same it has been necessary to submerge the paper for at least two minutes to insure adequate wetting on dry days. The use of pretreated paper, i. e., paper treated with recording solution prior to its utilization in the recording apparatus, has heretofore proven impractical for the electrolytic treatment when subjected to moistening by water in the absence of a wetting agent. Differently stated, the wetting agent causes the water to penetrate pretreated paper more rapidly than the solution penetrates untreated paper. Moreover, an additional function of the wetting agent is to cause the recording solution on the surface of the paper to continue penetration until saturation occurs, where excess liquid is available on the paper surface. Any remaining excess of liquid is removed by any conventional expedient, such as by a doctor blade or a preheater.

An undue amount of liquid on the paper may function to cause blurring at the instant of printing. Where the interval between paper wetting and facsimile printing is comparatively long, the tendency is for the paper to become partially dry, causing streaking and paper scuffing when the printing is applied. The wetting agents serve to retard the rate of drying at this stage of the operation.

Glycols and other high boiling solvents also retard drying at room temperature and improve wetting, but they are not as effective as wetting agents, thereby necessitating much greater concentrations. If the damp paper, after being subjected to recording, is passed over a hot roller for the purpose of drying and ironing it, the glycols require a greater extent of heating, since at higher temperatures they are more effective than wetting agents as drying retardants. Wetting agents similarly are advantageous in the case of pretreated damp paper which is stored in a moisture-proof container, to be later positioned in a slotted container at the point of unrolling at the recorder.

An element which materially affects color intensity is the amount of diazonium compound formed electrolytically. It will be appreciated, in this respect, that the halftones of photographs are reproduced by variations in color intensity caused by variations in signal strength. The extent of diazonium compound formation, and therefore color intensity, assumes the characteristics of a linear function of the current flow,

except at very low currents where the color intensity drops sharply due to the so-called threshold value effect. In view thereof, reducing agents as well as high alkalinity serve to detract from the light tones. This threshold effect may be compensated for by resort to color-deepening chemicals, illustrated by urea, thiourea, and di-cyandiamidine, which improve the halftone characteristics by accentuating the light tones.

Other substances which tend to deepen the color or improve background permanency are barium and calcium chlorides which may be substituted in part, or entirely, for sodium chloride as the electrolyte. Such substitution may, however, not be without its shortcomings in view of the possibility that the solubility of the dye chemicals may be lowered and on occasion objectionable sludges may be formed.

Through the choice of primary amines and coupling compounds used a great variety of colors may be obtained, although orange, red and purple shades predominate. In general, the orange dyes give recordings whose backgrounds are more permanent without washing than the reds, purples or blues. Furthermore, it has been found that alpha-naphthalene compounds generally give darker colors, but with less permanent backgrounds, than the corresponding beta compounds.

On the question of background permanence, some amines and coupling compounds, in some cases those having two or more amino or hydroxy groups on the same benzene or naphthalene ring, may manifest an undue tendency to air oxidation and it may be desirable as a general expedient to wash recordings made through the use of such reagents within a few hours after such recordings in order to prevent excessive background darkening on storage. Taken as a whole, the remaining amines and coupling compounds give satisfactory recordings which retain their white backgrounds, or at least do not darken sufficiently to impair their legibility and utility when stored several years in a file or holder.

As previously suggested, various chemicals function to retard background darkening, among which are glycols. These substances are used in the proportion of approximately 100 cc. per liter of solution. In some cases, they reduce darkening due to the slow reaction during storage, but are not as effective with respect to darkening which results from light exposure.

Reducing agents, such as sodium hydrosulphite ( $\text{Na}_2\text{S}_2\text{O}_4 \cdot 2\text{H}_2\text{O}$ ) and acetaldehyde sodium bisulphite ( $\text{NaOSO}_2 \cdot \text{CHOHCH}_3$ ) tend to retard the darkening action of light, but may not preclude slow darkening. Quantities varying from 0.002 to 0.01 mol per liter have been utilized with effective results within the scope indicated. The reducing agents specified are merely illustrative, since other reducing agents have a similar effect. Such other reagents are tartrates, formates, sulphites, thiosulphites, other hydro-sulphites than sodium, mentioned above, etc.

The effect of alkalinity upon background darkening has already been recited, and the same applies to the optimum range of pH between 9.5 and 11.0, especially where sodium chloride is used as the electrolyte. Higher pH may cause weakening and decomposition of the paper, while lower pH may result in partial oxidation and partial self-diazotization of the amines. The pH of the paper before treatment with the solution is known to effect the final alkalinity of the treated pa-

per; therefore, if an acid paper is used, the alkalinity of the solution should be increased to compensate therefor.

Complex cyanides of iron, chromium, or other metals, in some instances improve the fastness of the dye records to washing and deepen the shade, or even alter the dye color. Noteworthy is the fact that the dyes are on the whole distinctly faster to washing than the intermediates from which they are formed. As a result of this, washing may be resorted to for removing unused chemicals from the unrecorded areas, thereby leaving intact the dyes corresponding to the subject of transmittal. As a general rule, recordings intended to be washed should preferably be made at a pH range of 8.0 to 10.0 within the broader range of 9 to 11.5; in this way advantage is taken of the greater color strength and increased fastness during such pH range. Urea, thiourea, and dicyandiamidine increase the fastness to washing. Thus these compounds serve the dual function of improving color strength as well as color fastness.

The minimum current which is required to produce a faint color is referred to as the threshold value. Before diazotization can take place, the initial alkalinity of the wet paper must be overcome. If reducing agents are present they are oxidized by part of the current, leaving less for acidification and diazotization. Thus the reducing agents referred to hereinabove show this threshold value effect. With neutral solutions or in the absence of reducing agents, small stray currents cause streaks and spots of color on unrecorded areas, thereby detracting from the appearance of the recordings and in some cases seriously interfering with the legibility of the small type.

The application of a constant negative potential to the printing mechanism has an effect analogous to that of high alkalinity in preventing streaks due to stray currents, since the positive facsimile signals must overcome this negative voltage before color appears. This expedient is, however, not without some difficulties in the way of an increased rate of corrosion of the negative electrode, and in the case of certain metals produces a pale negative recording on the back of the paper. It may also tend to eliminate the lighter shades in reproduction of photographs.

Illustrative of desirable embodiments of the invention, the following examples are presented:

*Example 1*

| Name and Use | Mols per Liter | Grams per 250 Liters |
|--------------|----------------|----------------------|
|--------------|----------------|----------------------|

PRE-MIXED INGREDIENTS

|                                         |      |        |
|-----------------------------------------|------|--------|
| Benzidine-3,3'-disulphonic Acid (amine) | .015 | 1634.5 |
| Acetosacetanilide (coupler)             | .002 | 88.5   |
| Schaeffer's Salt (coupler)              | .003 | 231.0  |
| Chromotropic Salt (coupler)             | .010 | 1248.7 |
| Sodium Hydrosulphite (auxiliary)        | .003 | 157.5  |
| Urea (auxiliary)                        | .010 | 150.2  |
| Sodium Chloride (electrolyte)           | .450 | 6576.1 |

SEPARATE MIXTURE

|                                                               |      |                        |
|---------------------------------------------------------------|------|------------------------|
| Sodium Hydroxide (alkali)                                     | .061 | 620.6 or 6.10 liters.  |
| Sodium Nitrite (nitrite)                                      | .060 | 1035.2 or 3.00 liters. |
| Sodium salt of aryl alkyl polyether sulfonate (wetting agent) | .08% | 750 cc.                |

*Example 2*

|                       | Name                            | Mols per Liter | Grams per Liter |
|-----------------------|---------------------------------|----------------|-----------------|
| PRE-MIXED INGREDIENTS |                                 |                |                 |
| 5                     | Benzidine-3,3'-disulphonic Acid | .015           | 6.538           |
|                       | Chromotropic Salt               | .015           | 6.000           |
| 10                    | Barbituric Acid                 | .004           | 0.512           |
|                       | Sodium Hydrosulphite            | .0028          | 0.588           |
|                       | Dicyandiamidine Sulphate        | .0010          | 0.316           |
|                       | Thiourea                        | .0010          | 0.076           |
|                       | Sodium Carbonate                | .030           | 3.721           |
|                       | Sodium Chloride                 | .300           | 17.536          |

SEPARATE MIXTURE

|    |                              |      |          |
|----|------------------------------|------|----------|
| 15 | Sodium Hydroxide, 2.5 Normal | .050 | 20.0 cc. |
|    | Sodium Nitrite, 5.0 Molal    | .074 | 14.8 cc. |

It will be noted in the above examples that while 20 the ingredients in each instance are separated into two groups, this is primarily indicative of a desirable expedient for packaging or storing the reagents prior to usage. However, considering the 25 compositions from the standpoint of their substantive content, they comprise the reagents specified in both groups.

As illustrative of the preparation of the composition of Example 1, the proper amounts of each 30 of the pre-mixed ingredients are weighed, and all are thoroughly mixed mechanically. A convenient method utilizes an inclined rotating drum containing pebbles or metal balls to break up any lumps in the chemicals. The mixture may be stored in bulk or packed in small packages each 35 containing the required quantity.

Since measuring liquids is much more convenient than weighing solids, it is advisable to use concentrated stock solutions of sodium hydroxide and sodium nitrite instead of the corresponding 40 solids. Approximately 2.5 normal sodium hydroxide (102 grams per liter) and 5.0 normal sodium nitrite (345 grams per liter) are adequate. The wetting agent is already in liquid form.

The composition adapted for electrolytic diazotizing and coupling is prepared by dissolving the 45 pre-mixed chemicals and sodium hydroxide in approximately three-fourths the required water, adding sodium nitrite and the remaining water, and filtering or decanting to remove sediment.

50 The wetting agent may be added at any time during or after the preparation, and varies in amount with operating conditions, although it is not critical.

The following table is indicative of expedient 55 amounts of each component utilizable in a recording solution, based upon the two different unit volumes, namely, the quart and the liter:

| 60 | Total Volume of Recording Solution | Pre-mixed Ingredients |       | Sodium Hydroxide (2.50 Normal) cc. | Sodium Nitrite (5.0 Normal) cc. |
|----|------------------------------------|-----------------------|-------|------------------------------------|---------------------------------|
|    |                                    | grams                 | cc.   |                                    |                                 |
|    | 1 quart                            | 38.181                | 32.50 | 23.091                             | 11.356                          |
| 65 | 1 liter                            | 40.346                | 34.34 | 24.400                             | 12.000                          |

Wetting agent—0.0 to 3 cc. of 25% solution per liter of recording solution.

In preparing the composition of Example 2, 70 the ingredients of the pre-mixed portion, containing all of the reagents except sodium hydroxide and sodium nitrite, may be mixed and ground together dry and stored in bulk. At the time that the reacting composition is prepared, the sodium hydroxide and sodium nitrite are added in ap-

properite proportion. A desirable pH for the composition when the respective portions have been admixed is between 10.75 and 11.0.

Additional examples are as follows:

*Example 3*

INGREDIENTS

| No. | Name                                   | Chemical Formula | Use                                             | Amount used per liter of solution |
|-----|----------------------------------------|------------------|-------------------------------------------------|-----------------------------------|
| I   | Orthotolidine 2-2' disulphonic acid    |                  | Amine                                           | 5.054 grams.                      |
| II  | Chromotropic Salt                      |                  | Coupling Compound                               | 3.640 grams.                      |
| III | Sodium Hydroxide (Normal solution)     | NaOH             | To dissolve (I) and make the solution alkaline. | 52 cc.                            |
| IV  | Sodium Nitrite (twice normal solution) | NaNO2            | To diazotize (I)                                | 15 cc.                            |
| V   | Sodium Chloride (Common salt)          | NaCl             | Electrolyte to permit current to flow.          | 52.5 grams.                       |
| VI  | Water                                  | H2O              | To total volume of 1000 cc.                     |                                   |

In the preparation of the solution, (I), (II), (III) and (V) are dissolved in about 800 cc. water. Since the commercial product (I) contains ammonia and some insoluble matter, the solution is filtered, and (IV) and the remaining water are then added.

The formula of the dis-azo dye formed is as follows:



*Example 4*

INGREDIENTS

| No. | Name                                   | Chemical Formula | Use                                   | Amount used per liter of solution |
|-----|----------------------------------------|------------------|---------------------------------------|-----------------------------------|
| I   | Sodium Naphthionate                    |                  | Amine                                 | 7.352 grams.                      |
| II  | Phloroglucinol                         |                  | Coupling Compound                     | 1.280 grams.                      |
| III | Sodium Hydroxide (normal solution)     | NaOH             | To make the solution alkaline         | 40 cc.                            |
| IV  | Sodium Nitrite (twice normal solution) | NaNO2            | To diazotize (I)                      | 15 cc.                            |
| V   | Sodium Chloride                        | NaCl             | Electrolyte to permit current to flow | 52.5 grams.                       |
| VI  | Water                                  | H2O              | To total volume of 1000 cc.           |                                   |

The solution is prepared similarly to Example 3, except that it is clear and does not require filtration. The same recording procedure gives orange-brown recordings on a white background, which turn pale yellow on exposure to light, and

behave like Example 3 recordings when washed. The dye is a mono azo dye, as follows.



## Example 5

## INGREDIENTS

| No. | Name                                   | Chemical Formula | Use                         | Amount used per liter of solution |
|-----|----------------------------------------|------------------|-----------------------------|-----------------------------------|
| I   | 4-Acetylaminio-1-7-Cleve's Acid        |                  | Amine                       | 9.228 grams.                      |
| II  | Gamma Acid                             |                  | Coupling Compound and Amine | 2.390 grams.                      |
| III | Sodium Hydroxide (Normal solution)     | NaOH             |                             | 70 cc.                            |
| IV  | Sodium Nitrite (twice normal solution) | NaNO2            |                             | 15 cc.                            |
| V   | Sodium Chloride (common salt)          | NaCl             |                             | 25.6 grams.                       |
| VI  | Water                                  | H2O              |                             | To total volume of 1000 cc.       |

The solution is prepared as in Examples 3 and 4, filtration being unnecessary. Excellent dark purplish-brown recordings on a white background are obtained. On standing, even in the dark, the background gradually becomes pale purple, but if the freshly made recording is washed with water the background darkens much more slowly and to a far lesser extent than that of unwashed recordings. The dye is a mixture, but consists mostly of the following:



Irrespective of the predetermined coloration to be obtained, dependent upon the reagents utilized, the supporting material, such as the paper, after having been appropriately treated with the reagents, is passed through the facsimile recorder in wet or moist condition. A desirable facsimile recorder which may be utilized is the bar-helix type, the bar servicing as the anode and the helix providing the cathode. However, it is apparent that the performance of the recording is not restricted to the use of any particular type of apparatus.

Upon contact with the printing electrodes of the recorder, the diazonium compound is formed, which couples with the coupling component present. Desirably, the treated or sensitized paper is fed continuously from a roll. Where the paper has not been sensitized, it is initially fed from the roll through the appropriate immersion bath for impregnation with the dye intermediates and auxiliary compounds, the excess immersion solution removed, and the paper passed directly to the recorder.

The reference to paper as the supporting material or carrier has been recited solely by way of illustration. Substantially any fibrous material capable of being dyed by an azo compound is within contemplation, including such materials as fabric, cloth, and other types of cellulosic sheets, regenerated or otherwise. Quite desirable results have been obtained with an all-rag sheet, surface-sized with glue-formaldehyde in order to impart adequate wet strength. Similarly, good results have been obtained with partially parchmentized wood pulp paper. In the case of pa-

25 pers which are too highly sized, wetting agents are employed to facilitate quick penetration of the solution; from 0.5 to 1.5 grams of wetting agent solids per liter of recording solution is usually sufficient for this purpose. Among the 30 effects produced are more rapid solution penetration into the paper and slower drying after leaving the treating bath.

Most all-sulphite papers are too weak when wet to be used on electrolytic bar-and-helix facsimile 35 recorders. When treated with urea-formaldehyde resins, sulphite paper increases in wet strength to the point where it becomes usable, although the tendency of formaldehyde to combine with the amine before diazotization weakens 40 the recorded color. If a sulphite with a fairly high initial wet strength is used, a moderate treatment gives adequate strength without excessive color-weakening. The treatment is preferably applied to the unsized paper.

Effective results may be obtained by combining formaldehyde and urea with the recording solution which has been freshly prepared, glycols being included to "stabilize" the initial resins formed. However, such solutions are not particularly stable when retained in storage for several days, since a substantial proportion of the 50 amine content is consumed, thereby resulting in a decrease in recorded color intensity. Freshly prepared solutions of this type utilized in obtaining dry pre-treated paper (paper which has been treated with the reagent solution and dried preliminary to its utilization as a recording sheet) may "set" the resin, and the dry storage conditions serve to prevent or minimize the relatively slow chemical reaction between the formaldehyde resin and the amine.

After subjecting the sheet to electrolytic treatment, especially where facsimile recording is involved, the carrier in a dry state is desirably kept in a folder protected from exposure to light. Although there may be a slight decoloration of the background after several hours' exposure to daylight, this does not seriously affect the utility of the article. Washing the freshly recorded sheets thoroughly with water at the most only slightly weakens the coloring of the dye which has been formed; at the same time, such washing substantially improves the permanence of the background.

Under preferred conditions of operation, the re-

cording paper, after having passed through the facsimile receiver may be subjected to a fixing bath for the purpose of rendering the dye more permanent in nature and/or to aid in the preservation of the white or neutral characteristic of the background. The paper is then desirably washed, as above indicated, to remove any chemicals which remain in the undiazotized portions of the paper in order to thereby minimize any tendency toward gradual fading of the color produced or darkening of the background when the recorded copy is exposed to light and/or air.

In preparing the various reagent solutions for utilization to saturate or impregnate the supporting material, certain precautions and details of procedure may be advisable, dependent upon the particular circumstances involved. Thus, where all the ingredients of a solution are neutral or alkaline upon their being dissolved in water, they may all be dissolved together. The sodium and potassium salts of amino- or hydroxy-naphthalene sulphonic acids fall in this class. Where the amines, coupling compounds, or other ingredients are free acids as distinguished from sodium or potassium salts, it is necessary to omit the sodium nitrite from the solution until all the acidic compounds have been dissolved by the excess alkali required to give the proper final alkalinity. Failure to observe this precaution results in the formation of diazonium compounds in the acidic zone adjacent to each dissolving crystal of the acidic compounds, with subsequent coupling and dye formation when the diazonium compound has reached the alkaline zone. Such solutions discolor any paper that is treated with them.

On storage, the solutions may tend to darken because of auto-oxidation of some of the ingredients, especially if exposed to light in clear bottles and to air in partly emptied bottles; sometimes this oxidation causes the formation of sediment, even though the solution was originally filtered. Nevertheless, good recordings have been obtained with some year-old solutions, at a slight sacrifice in background permanence. Solutions that have become dark on standing may be restored to their original color (amber, clear brown, or red) by the addition of small amounts of sodium hydrosulphite.

Where the reagents are retained in their solid form, all or part of them may be packed in glass bottles, waterproof fiber or tin cans, or any other suitable containers, so that the user merely dissolves the contents of one or two containers in water, mixes the two solutions if two containers are needed, and adds more water until the required volume of solution is reached. In those cases where impurities in the water or in the chemicals cause sediment to form, the solution may either be filtered, or allowed to stand several hours to permit the precipitate to settle, so that the clear liquid may be decanted.

By separating the rest of the ingredients (in the containers for dry solids) by layers of salt (which constitutes the greater part of the volume of dry ingredients), any tendency for slow chemical reactions between the ingredients during dry storage is avoided, since salt is inert with respect to the other ingredients. In case any of the dry solids cake in the container, they may be rinsed into the solution with water.

In preparing the carrier material, illustrated by paper, for electrolytic facsimile recording, alternative procedures are available. These may be listed as involving the following three meth-

ods: (a) chemical treatment of paper at the recorder, (b) damp pre-treated paper requiring no treatment at the recorder, and (c) dry pre-treated paper requiring treatment with water at the recorder.

Considering the recorder-treated paper, the untreated paper is fed through an immersion bath or over wet rollers, where it becomes saturated with a solution of the recording chemicals. After removal of excess solution by doctor blades, and of excess moisture, by natural evaporation or by a heated roller, the wet paper passes through the facsimile recording mechanism. This method is more convenient experimentally, since both recording and paper treatment are combined in one operation. It has the advantage of lower cost for chemicals and paper due to elimination of pre-treating costs, and is excellent for use in commercial high speed recording where properly instructed operators give the recorders frequent attention. It may not be entirely suitable for home reception of facsimile broadcasting, since it involves the handling in the home of chemicals which require an element of care and precaution to avoid spilling, discoloring of furniture and clothes.

With respect to the damp pre-treated paper (b), the treating and recording operation may be separated, the paper being treated and rewound while still wet, and delivered in sealed moisture-proof containers to the recorders. When required for use, the wet roll of paper is transferred to a slotted container in a recorder, from which it is fed to the printing mechanism. This method imposes less strain on the paper than any other wet electrolytic recording method, as the damp paper does not stretch or wrinkle between the slot and the printing point. Consequently much weaker paper may be used. Quick starting with intermittent operation, a desirable feature in telegraph offices, is easily accomplished by manually pulling out the paper for a distance equal to that between the container slot and the printing point. The inclusion of wetting agents in the treating solution eliminates excessive drying of the paper between the container slot and the printing point during normal operation.

The shelf life of damp treated paper varies with the chemicals used and with the alkalinity. Usually, the interval within which it should be utilized extends for slightly less than three months from the time that the paper has been prepared. Refrigeration, even with Dry Ice, does not harm either the chemicals or the paper and desirably functions to increase the shelf life. A temperature just above the freezing point of water has shown indications of providing the best results, and avoids the necessity for thawing the paper before use.

Both metal foil wrappers and tin cans with or without internal coating have been utilized for packaging damp pretreated paper. In the case of the cans, a tendency toward rusting is manifested, and for this reason the metal foil is preferable. Tin foil gives better results than either lead or aluminum foil, but it is believed that the moisture retention may not be as effective as in the case of a sealed metal can. The acidity of asphalt-laminated paper causes discoloration of the outer layers of the pre-treated paper. Preferred results may be obtainable by use of a metal foil wrapper on the treated roll of paper, together with a waxed fiber can, desirably with a screw top that is waxed after being closed.

In accordance with the above description, it

will be apparent that sheets of the carrier material may be impregnated with one or more of the various ingredients and solutions within the purview of the invention, and then permitted to dry. When the carrier is dry, it is essentially non-conducting and is not in proper condition to be operated upon by the passage of electric current. To utilize the same, it may be humidified or dampened by any appropriate means, such as by steam or water vapor, in order to increase the conductivity thereof and render it utilizable in the facsimile receiving machine. By so preparing the sheets of chemically treated paper in a dry form as separate rolls, it is possible to use this treated or sensitized paper by merely subjecting the same 15 utilized:

While several definite examples have been presented by way of illustration of the features of the invention, the scope thereof is in no sense restricted to the use of such examples or the particular ingredients specified in such examples. As a general indication, substantially any of the desirable amino compounds listed above may be utilized with substantially any of the coupling compounds which have been set forth. In further illustration of solutions which have been found to produce very favorable results for facsimile recording especially with respect to background permanence, the following is presented as indicative of the amine and coupling compound

Amine (listed first) and Coupler (listed directly beneath amine)

|                                                                                                         | Concentration of Ingredients in<br>Mols/liter— $\text{NaNO}_2=0.03$ |         |               |               |
|---------------------------------------------------------------------------------------------------------|---------------------------------------------------------------------|---------|---------------|---------------|
|                                                                                                         | Amine                                                               | Coupler | $\text{NaOH}$ | $\text{NaCl}$ |
| 1-amino benzene-4-sulphonic acid **                                                                     | .032                                                                | .010    | .090          | 1.000         |
| 1,3,5-trihydroxybenzene                                                                                 |                                                                     |         |               |               |
| 1-amino benzene-4-sulphonic acid **                                                                     | .030                                                                | .015    | .080          | 1.000         |
| 2-naphthol-6-sodium sulphonate                                                                          |                                                                     |         |               |               |
| 1-amino benzene-4-sulphonic acid **                                                                     | .030                                                                | .015    | .090          | 1.000         |
| 2-naphthol-3,6-disodium disulphonate                                                                    |                                                                     |         |               |               |
| 1-amino benzene-4-sulphonic acid **                                                                     | .030                                                                | .015    | .080          | 1.000         |
| 2-naphthol-6,8-disodium disulphonate                                                                    |                                                                     |         |               |               |
| 1-methyl-2-amino benzene-5-sodium sulphonate **                                                         | .030                                                                | .010    | .040          | 1.000         |
| 2-hydroxy-3-naphthoic acid                                                                              |                                                                     |         |               |               |
| 2,4-diaminodiphenyl-2,2'-disulphonic acid **                                                            | .015                                                                | .010    | .060          | 1.000         |
| 1,3,5-trihydroxybenzene                                                                                 |                                                                     |         |               |               |
| 4,4'-diaminodiphenyl-2,2'-disulphonic acid **                                                           | .015                                                                | .010    | .060          | 1.000         |
| 2-hydroxy-3-naphthoic acid                                                                              |                                                                     |         |               |               |
| 4,4'-diaminodiphenyl-2,2'-disulphonic acid **                                                           | .015                                                                | .010    | .060          | 1.000         |
| 2-naphthol-6-sodium sulphonate                                                                          |                                                                     |         |               |               |
| 4,4'-diaminodiphenyl-2,2'-disulphonic acid **                                                           | .015                                                                | .015    | .060          | 0.910         |
| 2-naphthol-3,6-disodium disulphonate                                                                    |                                                                     |         |               |               |
| 4,4'-diamino-3,3'-dimethyl-6,6'-disulphodiphenyl or 4,4'-diamino-5,5'-dimethyl-2,2'-disulphodiphenyl ** | .015                                                                | .015    | .060          | 1.000         |
| 3-diethylamino-1-phenol                                                                                 |                                                                     |         |               |               |
| 4,4'-diamino-3,3'-dimethyl-6,6'-disulphodiphenyl or 4,4'-diamino-5,5'-dimethyl-2,2'-disulphodiphenyl ** | .016                                                                | .015    | .067          | 1.000         |
| 2-naphthol-6-sodium sulphonate                                                                          |                                                                     |         |               |               |
| 4,4'-diamino-3,3'-dimethyl-6,6'-disulphodiphenyl or 4,4'-diamino-5,5'-dimethyl-2,2'-disulphodiphenyl ** | .016                                                                | .015    | .082          | 0.888         |
| 2-naphthol-3,6-disodium disulphonate                                                                    |                                                                     |         |               |               |
| 1-naphthylamine-4-sodium sulphonate **                                                                  | .016                                                                | .015    | .052          | 0.888         |
| 2,4-dihydroxyphenylmethylketone                                                                         |                                                                     |         |               |               |
| 1-naphthylamine-4-sodium sulphonate **                                                                  | .030                                                                | .015    | .030          | 0.910         |
| 1,3,5-trihydroxybenzene                                                                                 |                                                                     |         |               |               |
| 1-naphthylamine-4-sodium sulphonate **                                                                  | .030                                                                | .010    | .040          | 1.000         |
| 3-diethylamino-1-phenol                                                                                 |                                                                     |         |               |               |
| 1-naphthylamine-4-sodium sulphonate **                                                                  | .030                                                                | .015    | .050          | 1.000         |
| 1-hydroxy-2-naphthoic acid                                                                              |                                                                     |         |               |               |
| 1-naphthylamine-4-sodium sulphonate **                                                                  | .030                                                                | .010    | .030          | 0.910         |
| 2-naphthol                                                                                              |                                                                     |         |               |               |
| 1-naphthylamine-4-sodium sulphonate **                                                                  | .030                                                                | .015    | .040          | 1.000         |
| 2-naphthol-3,6-disodium disulphonate                                                                    |                                                                     |         |               |               |
| 1-naphthylamine-4-sodium sulphonate **                                                                  | .030                                                                | .015    | .035          | 0.875         |
| 8-hydroxyquinoline                                                                                      |                                                                     |         |               |               |
| 1-naphthylamine-5-sulphonic acid **                                                                     | .030                                                                | .015    | .035          | 1.000         |
| 8-hydroxyquinoline                                                                                      |                                                                     |         |               |               |
| 2-naphthylamine-1-sulphonic acid **                                                                     | .033                                                                | .010    | .073          | 0.897         |
| 1,3,5-trihydroxybenzene                                                                                 |                                                                     |         |               |               |
| 2-naphthylamine-1-sulphonic acid **                                                                     | .032                                                                | .010    | .042          | 1.000         |
| 1-hydroxy-2-naphthoic acid                                                                              |                                                                     |         |               |               |
| 2-naphthylamine-1-sulphonic acid **                                                                     | .030                                                                | .015    | .070          | 0.900         |
| 2-naphthol                                                                                              |                                                                     |         |               |               |
| 2-naphthylamine-1-sulphonic acid **                                                                     | .032                                                                | .015    | .05714        | 1.000         |
| 2-hydroxy-3-naphthoic acid                                                                              |                                                                     |         |               |               |
| 2-naphthylamine-4,8-disulphonic acid **                                                                 | .032                                                                | .010    | .100          | 1.000         |
| 2-naphthol-3,6-disodium disulphonate                                                                    |                                                                     |         |               |               |
| 2-naphthylamine-6,8-disulphonic acid **                                                                 | .033                                                                | .015    | .066          | 0.874         |
| 1,3,5-trihydroxybenzene                                                                                 |                                                                     |         |               |               |
| 2-naphthylamine-6,8-disulphonic acid **                                                                 | .033                                                                | .010    | .096          | 0.876         |
| 3-diethylamino-1-phenol                                                                                 |                                                                     |         |               |               |
| 2-naphthylamine-6,8-disulphonic acid **                                                                 | .033                                                                | .015    | .101          | 0.869         |
| 1-hydroxy-2-naphthoic acid                                                                              |                                                                     |         |               |               |
| 2-naphthylamine-6,8-disulphonic acid **                                                                 | .033                                                                | .010    | .098          | 0.874         |
| 2-naphthol                                                                                              |                                                                     |         |               |               |
| 2-naphthylamine-6,8-disulphonic acid **                                                                 | .033                                                                | .015    | .101          | 1.000         |
| 2-naphthol-6-sodium sulphonate                                                                          |                                                                     |         |               |               |
| 2-naphthylamine-6,8-disulphonic acid **                                                                 | .033                                                                | .015    | .081          | 0.900         |
| 2-naphthol-8-sulphonic acid                                                                             |                                                                     |         |               |               |
| 2-naphthylamine-6,8-disulphonic acid **                                                                 | .033                                                                | .015    | .116          | 0.854         |
| 2-naphthol-3,6-disodium disulphonate                                                                    |                                                                     |         |               |               |
| 2-naphthylamine-6,8-disulphonic acid **                                                                 | .033                                                                | .015    | .101          | 0.839         |
| 8-hydroxyquinoline                                                                                      |                                                                     |         |               |               |
|                                                                                                         | .033                                                                | .010    | .096          | 1.000         |

<sup>1</sup> Potassium hydroxide was used here instead of sodium hydroxide.

to an appropriate degree of moisture in order that the current may pass therethrough and accordingly cause a dye to appear thereon, corresponding with the electric impulses from a transmitting source.

As pointed out hereinabove, the details of the facsimile recorder from a structural standpoint do not constitute an element of the present invention. The nature of the electrodes, however, may be of interest, although it is not contemplated

that they should be of the type which enter into the compositions of the dyes formed during electrolytic diazotization. Among the contact electrodes which have been utilized are stainless steel, tungsten, molybdenum, platinum, and platinum-iridium. In general, the hard, inert metals such as platinum-iridium and the stellites provide the best results as recording anodes. Non-magnetic stainless steels similarly give good results, but the colors differ from that produced by the platinum or stellite, and may be less attractive in appearance, possibly attributable to collateral reactions involving the iron. Ordinary steels which are strongly attracted by magnets do not permit any diazotization reaction, but, on occasion, they produce a moderately pale green recording which is believed to result from oxidation of the intermediates. In the case of alloy electrodes, the percentage of azo color resulting from diazotization appears to increase as the magnetic characteristics of the alloy decrease. By way of explanation as a plausible hypothesis, it may be that the magnetic metals create a strong magnetic field when the current passes, and this magnetic field orients the electrically charged ions in such directions and in such manner that they preclude the possibility of diazotization.

Copper alloys and electrodes generally made from copper or nickel tend to inhibit electrolytic diazotization recording and are, therefore, as a general matter not satisfactory for use as recording anodes, although they give excellent results as cathodes. In this category is the beryllium-copper alloy.

Tungsten generally provides satisfactory recordings, but it manifests a tendency to build up a non-conductive coating, thereby requiring more signal current for effective recording as well as the occasional necessity for reversing the current during a brief interval in order to remove the coating.

The tendency is for the cathode to indicate substantially less electrolytic wear than the anode, since it is attacked only by nascent hydrogen and by increased alkalinity at the time of current flow. With a bar-helix type of recorder, the cathode is desirably in wire form, and the principal wear is due to abrasion which gradually renders the wire flat. The beryllium-copper cathode necessitates more frequent replacement than the anode when the latter is either platinum-iridium or stellite. A cathode helix wire of stellite may outlast several stellite or platinum-iridium anode printer bars.

It will be apparent from the foregoing that the use of compositions within the scope of the present disclosure enables the production of dyes and pigments by subjecting solutions or mixtures of chemicals to electric current. Such dyes or pigments may be obtained in the form of a paste, powder, or as a liquid solution, and subsequently adapted for use as coloring paints, inks, etc., or for dyeing various materials. It is within the contemplation of the invention to produce such dyes or pigments by intermittent or continuous reaction. Materials such as clothing, piece goods, yarn, paper, and generally any fibrous material susceptible to dyes, and particularly azo dyes, fall within the purview of the present disclosure. They may be treated by immersion in a container filled with a solution of predetermined ingredients and subsequently subjecting such solution to the flow of an electric current in order that the dye may be fixed in or on the materials immersed therein; thus, the dye application may be in the

form of a surface coating or a dyeing within the fibrous structure. Definitely contemplated is the formation of the dye in situ.

While I have described my invention in accordance with preferred embodiments as to compositions, articles of manufacture, and procedure, it is apparent that many variations and modifications both as to procedural details, compositions of matter, and articles of manufacture may be made without departing from the scope of equivalents within the purview and spirit of the invention.

The term "facsimile" as used herein is intended to involve not only the reproduction on the recording material of a pre-existing subject, for example a photograph which is scanned and reproduced in accordance with the impulses emanating from the scanning operation, but also embraces the recording of subject matter in the process of creation or formation without a physically pre-existing subject. As illustrative of this latter category would be the recording of simply a mental preconception, for example a pattern or design, either of a single color and shades thereof, or multicolors, which is recorded in accordance with an appropriate manual or automatic variation of the electric impulses delivered to the electrodes. Similarly in this category is intended the recording of an arbitrary or haphazard design, pattern or other subject, for example one secured by haphazardly or arbitrarily varying electric impulses delivered to the electrode by punching keys on a master keyboard having suitable electrical connections, by manually or automatically varying resistance, or the like.

Having thus described the invention, what is claimed as new and desired to be secured by Letters Patent is:

40. 1. A fibrous sheet material for the electrolytic formation of an azo dyestuff thereon having the surface thereof uniformly treated with an aqueous solution of a dyestuff forming composition consisting substantially of a diazotizable primary amine, a sufficient quantity of an alkali metal nitrite to produce the nitrite ions necessary for diazotization of said amine under the influence of the electrolyzing current, a water soluble neutral inorganic salt in addition to said nitrite as the electrolyte in an amount to insure passage of the electrolyzing current, a sufficient quantity of an azo dye coupling component to couple with the diazonium compound when formed to produce an azo dye, and a quantity of alkali sufficient to impart to said composition a pH on the alkaline side to thereby preclude diazonium salt formation until the fibrous sheet material is subjected to the action of the electrolyzing current said fibrous sheet material being free from any azo dyestuff.

60. 2. The article as defined in claim 1 in which the solution has a pH ranging from 9 to 11.5.

3. The article as defined in claim 1 in which the diazotizable amine is an aromatic polyamine.

65. 4. The article as defined in claim 1 in which the composition contains a wetting agent to facilitate application of the composition to the fibrous sheet material.

70. 5. The article as defined in claim 1 in which the composition contains a compound to improve the color intensity of the azo dyes, said compound being selected from the class consisting of urea, thiourea and dicyandiamidine.

75. 6. The article as defined in claim 1 in which the ionizable nitrite is sodium nitrite, the elec-

troyte is sodium chloride and the alkali is caustic soda.

7. The article as defined in claim 1 in which the coupling component is alkaline reacting.

8. The article as defined in claim 1 in which the coupling component is acid reacting.

NELLIE W. SOLOMON,  
*Administratrix of Estate of Myer Solomon, Deceased.*

## REFERENCES CITED

The following references are of record in the file of this patent:

## UNITED STATES PATENTS

| Number    | Name            | Date          |
|-----------|-----------------|---------------|
| 168,466   | Edison          | Oct. 5, 1876  |
| 366,078   | Duisberg        | July 5, 1887  |
| 423,970   | Ulrich          | Mar. 25, 1890 |
| 440,953   | Majert          | Nov. 18, 1890 |
| 761,310   | Loeb            | May 31, 1904  |
| 1,646,296 | Kircheison      | Oct. 18, 1927 |
| 1,844,199 | Bicknell        | Feb. 9, 1932  |
| 1,857,230 | Zitscher et al. | May 10, 1932  |
| 1,880,449 | Hickman et al.  | Oct. 4, 1932  |
| 1,892,099 | Cornell         | Dec. 27, 1932 |
| 1,916,947 | Haendel         | July 4, 1933  |
| 1,970,539 | Bausch          | Aug. 31, 1934 |

| Number    | Name             | Date           |
|-----------|------------------|----------------|
| 2,008,966 | Powers et al.    | July 23, 1935  |
| 2,063,992 | Elsey            | Dec. 15, 1936  |
| 2,080,209 | Kappeler         | May 11, 1937   |
| 2,108,852 | Gettinger        | Feb. 22, 1938  |
| 2,112,864 | Pool et al.      | Apr. 5, 1938   |
| 2,138,572 | Etzelmiller      | Nov. 29, 1938  |
| 2,154,918 | Schneider et al. | Apr. 18, 1939  |
| 2,173,141 | Talmey           | Sept. 19, 1939 |
| 2,181,533 | Kline et al.     | Nov. 28, 1939  |
| 2,186,732 | Schneider et al. | Jan. 9, 1940   |
| 2,186,850 | Wilmanns et al.  | Jan. 9, 1940   |
| 2,286,662 | Weyde et al.     | June 16, 1942  |
| 2,306,471 | Solomon          | Dec. 29, 1942  |
| 2,309,492 | Albers et al.    | Jan. 26, 1943  |

## FOREIGN PATENTS

| Number | Country       | Date |
|--------|---------------|------|
| 13,343 | Great Britain | 1890 |

## OTHER REFERENCES

|                                                                                     |
|-------------------------------------------------------------------------------------|
| Color Index, pages 201, and 202, by F. W. Rowe, Jan. 1924.                          |
| The Aromatic Diazo Compounds, by Saunders, 1936, pages 50, 51, 102-104, and page 2. |
| Zeitschrift fur Elektrochemie, vol. X (1940) pages 236, 237 (an article by Lob).    |